

## UNITED STATES PATENT OFFICE

ERICH KAYSER, OF FRANKFORT-ON-THE-MAIN GRIESHEIM, GERMANY, ASSIGNOR TO  
I. G. FARBENINDUSTRIE AKTIENGESELLSCHAFT, OF FRANKFORT-ON-THE-MAIN,  
GERMANY

## METHOD OF BLEACHING VEGETABLE FIBROUS SUBSTANCES

No Drawing. Application filed November 22, 1929, Serial No. 409,179, and in Germany March 1, 1928.

This invention relates to improvements in the process of bleaching vegetable fibrous substances, for instance in the wood cellulose bleach.

5 When bleaching vegetable fibrous substances, especially wood cellulose by means of hypochlorite solutions as bleaching agents, experience has shown that the bleach at first proceeds rapidly, but subsequently is steadily retarded, the bleach progressing at definite speed according to the laws of monomolecular reactions. The progress in the bleaching effect as observed, as well as the consumption of chlorine from the solution corresponds 10 to these facts. The accumulation of incrustations originally contained in the untreated fibre and dissolved in the bleaching bath during the bleach entails, as we know, the danger of colloidal precipitations forming 15 upon the fibers, when the treated material in a subsequent stage of the process is washed out with water during the so-called dilution wash, thus increasing the contents of ashes in the bleached material to a relatively high 20 degree. Numerous propositions have been made to avoid this inconvenience; for instance, a method is known for carrying out the bleaching of cellulose according to the counter-current principle. According to 25 this method the material is impregnated with the bleaching solution, then, as far as possible, freed from the partially exhausted bleaching solution in a suitable concentrator and impregnated anew with a more concentrated 30 bleaching solution. However, in spite of certain advantages, this process presents the drawback of calling for repeated operations and above all of prolonged duration.

Now I have found that the bleaching 35 period can be considerably curtailed by lowering the temperatures of the individual bleaching solutions simultaneously with increasing the concentration in such a manner that the weakest bleaching solution (or final 40 solution) has the highest temperature of, say, about 25-35° C., whereas the strongest bleaching solution (or initial solution) is applied at, say, about 15-25° C. It is understood that also other ranges of temperatures 45 may be employed. The gradation of the con-

centration of the bleaching agent in the bleaching solution should be adjusted to the bleachability of the material to be treated. Thus, for difficultly bleachable materials the absolute concentrations should be higher and 55 the differences between the successive steps larger than for easily bleachable substances. I preferably subject the raw material to the bleaching treatment in the form of paste-board sheets. This bleaching method possesses 60 considerable advantages as the repeated concentration of the material is done away with.

Now I have found that the application of the counter-part principle in the bleach of 65 paste-board sheets by combining it with adapting the temperature of the bleaching solution inversely to its chlorine contents, entails a very great reduction of the bleaching period and a complete utilization of the 70 bleaching solution. For instance, a running sheet of cellulose paste-board is impregnated in three successive sections *a*, *b*, *c*, with bleaching solutions of different concentration. Thus the section *a* (comprising the 75 raw material) receives the bleaching solution *a'* containing a limited chlorine content, say, about 10 grams of available chlorine per liter, which is practically exhausted by interaction with the raw material. When the sheet advances to the place *b*, the stronger bleaching solution *b'* containing about 20 grams per liter of available chlorine is brought to react, then pressed out and is further employed 80 (its chlorine content being reduced to about 10 grams per liter) as a solution *a'* for the next batch. Finally the sheet reaches the position *c* where the strongest bleaching solution *c'* enters, showing an initial contents of 85 available chlorine of about 30 grams per liter, and, after having exercised its bleaching action, is pressed out and withdrawn forming now solution *b'* for the next batch. After having undergone this bleaching 90 treatment, during which the temperature of the solution is lowered while the available chlorine contents increases with each subsequent bleaching step, the material which no longer contains incrustations (the latter hav- 100

ing been carried away by the solutions  $a'$ ,  
 $b'$ ,  $c'$ ,) is thoroughly washed only once. The  
final product is a completely or partly  
bleached material, as desired, free from in-  
5 crustations, and this product is obtained  
within a considerably shorter time than  
formerly.

The improvement in the new bleaching  
process for paste-board sheets thus consists in  
10 combining the counter-current principle for  
the raw material and the bleaching solution,  
and adapting the temperatures and the con-  
centration of the bleaching solutions so as  
15 to regulate the temperature in an inverse  
sense to the chlorine contents in the bleach-  
ing solution. Said improvement affords, on  
the one hand, the advantage of the incrusta-  
tions being completely removed from the  
20 material under treatment by squeezing off  
the solutions, and, on the other hand, per-  
mits of accomplishing the bleach in the  
shortest time.

I claim:—

In the method of bleaching vegetable  
25 fibrous substances, especially wood cellulose,  
in which method the raw material is treated  
in form of a paste-board sheet and in counter-  
current with bleaching solutions of suc-  
cessively increasing concentration of available  
30 chlorine, the improvement which comprises  
adapting the temperature of the respective  
bleaching solutions inversely to the chlorine  
content of said bleaching solutions.

In testimony whereof, I affix my signature.  
35 ERICH KAYSER.

40

45

50

55

60

65